# EUROPEAN PATENT SPECIFICATION

(11) **EP 0 648 851 B1**
(45) Date of publication and mention of the grant of the patent: **14.07.1999**
(21) Application number: 94306632.4
(22) Date of filing: 09.09.1994
(51) Int. Cl.: C22C 33/02, C22C 38/60, B22F 9/08

(54) **Sulfur-containing powder-metallurgy tool steel article and its method of manufacture**
Artikel aus Schwefel enthaltenden Werkzeugstahlpulver und Verfahren zu seiner Herstellung
Article en poudre d'acier à outils contenant du soufre et son procédé de fabrication

(30) Priority: 27.09.1993 US 126562
(43) Date of publication of application: 19.04.1995
(73) Proprietor: CRUCIBLE MATERIALS CORPORATION, Syracuse, New York 13201-0977 (US)
(72) Inventor: Stasko, William, West Homestead, Pennsylvania 15120 (US); Pinnow, Kenneth E., Pittsburgh, Pennsylvania 15237 (US)
(74) Representative: Coxon, Philip

(56) References cited:
- EP-A- 0 183 666
- EP-A- 0 515 018
- DE-A- 4 040 030
- US-A- 3 598 567
- J.R.DAVIS ET AL 'METALS HANDBOOK' 1990 , ASM , OHIO 10th edition vol.1 * page 780 - page 791 * * page 780, column 3, line 5 - line 13 * table 1 ex. 7 * page 781, column 3, line 12 - line 24 * * page 783, column 1, line 10 - line 41 * * page 789, column 3, line 60 - page 790, column 3, line 7 *

## Description

### BACKGROUND OF THE INVENTION

### Field of the Invention

This invention relates to a tool steel article made of a hot worked powder metallurgy tool steel having higher than conventional sulfur content and a method for producing the same.

### Description of the Prior Art

Tool steels are used conventionally in the manufacture of tooling articles employed in both cutting and noncutting tooling applications. This includes the manufacture of broaches and hobs, as well as of rolls, punches and mold components. In these tooling applications, it is necessary that the tool steel have sufficient strength, toughness, and wear resistance to withstand the service conditions encountered in these typical applications. In addition, they must have adequate machinability and grindability to facilitate production of the desired tooling components.

It is known that the presence of sulfur in tool steels improves their machinability and grindability by forming sulfides that act as a lubricant between the cutting tools used to form the tool component and the chips removed from the steel during this operation. The sulfides also promote chip breaking during the cutting operation incident to tool manufacture to thereby further facilitate this operation.

The use of sulfur in amounts over about 0.10% is known to reduce the hot workability of conventional ingot-cast tool steels and adversely affect their mechanical properties, particularly their toughness. In conventional high sulfur containing tool steels, the sulfides are typically larger and elongated in the direction of hot working. Likewise, with conventional wrought tool steels, the primary carbides in the steel are strung out during hot working to form carbide stringers in the direction of working. The carbide stringers in these steels adversely affect mechanical properties, and their negative effects are so pronounced that they generally overshadow any adverse effects of the sulfides in this regard.

On the other hand, during the manufacture of high sulfur containing tool steel articles by a powder metallurgy practice wherein prealloyed particles of the steel are consolidated to achieve a fully dense article, the carbides are relatively small and well distributed compared to those in conventional tool steels. Because of the favorable size and distribution of the carbides achieved in these tool steels, the adverse effects of the carbide stringers encountered in conventional wrought steel are avoided. The properties of the powder metallurgy produced tool steels are therefore more sensitive to changes in sulfur content and to the size and distribution of the sulfides introduced for the purpose of improving their machinability or grindability. For this reason, sulfur in amounts greater than about 0.07%, are generally not used in powder metallurgy produced tool steels because of the adverse effects of the sulfides on their mechanical properties, for example, as indicated by a decrease in the bend fracture strength of the steel. Powder metallurgy tool steel articles with higher sulfur contents would be more widely used, if the detrimental effects of sulfur on their mechanical properties could be avoided.

### SUMMARY OF THE INVENTION

It is accordingly a primary object of the present invention to provide a tool steel article produced from a hot worked powder metallurgy produced high sulfur tool steel wherein the presence of sulfur and resulting sulfides does not significantly adversely affect the mechanical properties while providing the beneficial effect of improved machinability and grindability.

A more specific object of the invention is to provide a tool steel article made from a hot worked high sulfur containing powder metallurgy produced tool steel wherein the presence of sulfur and resulting sulfides does not significantly degrade toughness, as exhibited by the bend fracture strength.

The invention provides a machinable powder metallurgy produced sulphur containing tool steel article in accordance with claim 1 or claim 2 of the appended claims.

Broadly, in accordance with the invention, there is provided a machinable powder-metallurgy produced sulfur-containing tool steel article comprising a hot worked, fully dense, consolidated mass of nitrogen-gas atomized, prealloyed particles of a tool steel alloy having a sulfur content of 0.10 to 0.30 weight percent with a maximum sulfide size controlled to be less than about 15 microns.

The tool steel alloy of the hot worked article may have a composition of a wrought high speed tool steel or of a wrought cold work tool steel to which sulfur has been intentionally added within a range of 0.10 to 0.30 weight percent. Broadly, the tool steel of the hot worked article may have in weight percent 0.80 to 3.00 carbon, 0.20 to 2.00 manganese, 0.10 to 0.30 sulfur, up to 0.04 phosphorus, 0.20 to 1.50 silicon, 3.00 to 12.00 chromium, 0.25 to 10.00 vanadium, up to 11.00 molybdenum, up to 18.00 tungsten, up to 10.00 cobalt, up to 0.10 nitrogen, up to 0.025 oxygen, and balance iron and incidental impurities. Tungsten may be substituted for molybdenum in the stoichiometric ratio of 2:1.

The machinable powder-metallurgy produced sulfur-containing tool steel article may have a minimum transverse bend fracture strength of 3450 MPa (500 ksi) when heat treated to a hardness of 64 to 66 HRC. The article comprises a hot-worked, fully dense, consolidated mass of nitrogen gas atomized, prealloyed particles of a tool steel alloy of, in weight percent, 1.25 to 1.50 carbon, 0.20 to 1.00 manganese, 0.10 to 0.26 sulfur, up to 0.04 phosphorous, up to 1.00 silicon, 3.0 to 6.0 chromium, 4.0 to 6.0 molybdenum, 3.50 to 4.50 vanadium, 4.0 to 6.5 tungsten, up to 0.025 oxygen, up to 0.10 nitrogen and balance iron and incidental impurities. The article has a maximum sulfide size controlled to be less than about 15 microns.

Preferably, the sulfur content of the articles in accordance with the invention may be within the range of 0.14 to 0.26%.

The invention further provides a method for manufacturing a powder metallurgy sulfur containing tool steel article in accordance with Claim 4 or Claim 5 of the appended claims.

The invention includes a method for manufacturing a powder-metallurgy sulfur-containing tool steel article of a hot worked, fully dense, consolidated mass of nitrogen atomized, prealloyed particles of a tool steel alloy having a sulfur content of 0.10 to 0.30 weight percent with a maximum sulfide size controlled to be less than about 15 microns. In accordance with the method, prealloyed particles are produced by nitrogen gas atomization and are hot isostatically compacted to full density at a temperature of 1185°C (2165°F) and a pressure of 1035 MPa (15 ksi). The resulting compact is hot worked to a desired article shape at a temperature of 1121°C (2050°F) and the article is then annealed.

The method in the invention may also be applied to prealloyed particles of a tool steel alloy of the composition, in weight percent, 0.80 to 3.00 carbon, 0.20 to 2.00 manganese, 0.10 to 0.30 sulfur, up to 0.04 phosphorous, 0.20 to 1.50 silicon, 3.0 to 12.0 chromium, 0.25 to 10.0 vanadium, up to 11.0 molybdenum, up to 18.0 tungsten, up to 10.0 cobalt, up to 0.10 nitrogen, up to 0.025 oxygen, balance iron and incidental impurities.

The method of the invention may likewise be used with prealloyed particles of a tool steel alloy of the composition, in weight percent, 1.25 to 1.50 carbon, 0.20 to 1.00 manganese, 0.10 to 0.26 sulfur, up to 0.04 phosphorous, up to 1.00 silicon, 3.0 to 6.0 chromium, 4.0 to 6.0 molybdenum, 3.50 to 4.50 vanadium, 4.0 to 6.5 tungsten, up to 0.025 oxygen, up to 0.10 nitrogen, balance iron and incidental impurities.

Preferably, the sulfur content may be within the range of 0.14 to 0.26 weight percent.

In accordance with the invention, the carbon present in the alloy combines with chromium, vanadium, molybdenum and tungsten to form the desired dispersion of wear resistant carbides and to promote secondary hardening. Sufficient carbon is also present to provide for strengthening of the matrix of the steel. The sulfur present in the steel combines primarily with the manganese to produce manganese sulfides or manganese-rich sulfides which facilitate the machinability and grindability of the steel.

To achieve the properties needed in the powder metallurgy produced tool steel articles of this invention, it is essential that the high sulfur powder metallurgy produced tool steels used in their construction be hot worked after consolidation to achieve the high mechanical strength needed for tooling components. It is also essential that the production and processing conditions for the powder metallurgy produced tool steels used in the articles of this invention be controlled so that the sizes and distribution of the sulfides introduced by the sulfur additions do not significantly degrade mechanical properties. In the powder metallurgy produced tool steel used in the tool steel articles of this invention, this is achieved by maintaining the maximum size of the sulfides below about 15 µm in their longest dimension.

### DETAILED DESCRIPTION OF THE PREFERRED EMBODIMENTS

By way of demonstration of the invention, a series of experimental tool steels were made with varying sulfur contents and subjected to various mechanical property and machinability tests. Samples of several commercial powder metallurgy produced high speed tool steels were also subjected to the same tests for comparison. Except for sulfur content, the commercial powder metallurgy tool steels generally have the same nominal composition as the experimental tool steels. The actual chemical compositions of the experimental tool steels and of the commercially produced tool steels are given in Tables I and II.

**TABLE I**

| CHEMICAL COMPOSITION OF EXPERIMENTAL POWDER METALLURGY TOOL STEELS | | | | | | | | | | | | | | |
|---|---|---|---|---|---|---|---|---|---|---|---|---|---|---|
| Bar Number | Heat Number | C | Mn | P | S | Si | Ni | Cr | V | W | Mo | Al | N | O |
| 92-17 | 518-662 | 1.42 | 0.30 | 0.007 | 0.004 | 0.51 | - | 3.89 | 4.04 | 5.66 | 5.28 | 0.02 | 0.034 | 0.006 |
| 92-18 | 518-658 | 1.45 | 0.34 | 0.006 | 0.05 | 0.54 | - | 5.00 | 3.73 | 5.44 | 4.90 | - | 0.035 | 0.005 |
| 92-19 | 518-659 | 1.42 | 0.46 | - | 0.14 | 0.54 | - | 3.86 | 3.80 | 5.49 | 4.90 | - | 0.027 | 0.006 |
| 92-20 | 518-63 | 1.39 | 0.64 | 0.005 | 0.26 | 0.57 | - | 3.86 | 3.97 | 5.79 | 5.05 | - | 0.028 | 0.013 |

**Table II**

| CHEMICAL COMPOSITION OF COMMERCIAL HIGH SULFUR TOOL STEELS | | | | | | | | | | | | | |
|---|---|---|---|---|---|---|---|---|---|---|---|---|---|
| Bar Number | C | Mn | P | S | Si | Ni | Cr | V | W | Mo | Co | N | O |
| 92-79 | 1.41 | 0.69 | 0.022 | 0.230 | 0.52 | 0.20 | 3.88 | 3.98 | 5.41 | 5.27 | 0.33 | 0.03 | 0.013 |
| 92-81 | 1.42 | 0.73 | 0.018 | 0.230 | 0.55 | 0.22 | 3.89 | 3.99 | 5.27 | 5.18 | 0.33 | 0.05 | 0.014 |
| 92-77 | 1.41 | 0.74 | 0.022 | 0.220 | 0.54 | 0.16 | 3.89 | 4.01 | 5.41 | 5.13 | 0.34 | 0.05 | 0.014 |
| 92-78 | 1.40 | 0.68 | 0.018 | 0.240 | 0.55 | 0.11 | 3.90 | 3.90 | 5.40 | 5.13 | 0.13 | 0.06 | 0.018 |
| 92-78 | 1.45 | 0.67 | 0.016 | 0.230 | 0.54 | 0.17 | 3.87 | 3.87 | 5.42 | 5.15 | 0.27 | 0.05 | 0.016 |
| 92-74 | 1.41 | 0.65 | 0.022 | 0.210 | 0.55 | 0.17 | 3.89 | 3.94 | 5.46 | 5.14 | 0.26 | 0.04 | 0.012 |

The production conditions for the experimental tool steels were designed to minimize the size of the sulfides in the microstructure. They were produced from nitrogen gas atomized prealloyed powders produced from 136 kg (300-pound) induction melted heats. About 91 kg (200 pounds) of powder from each heat were screened to -16 mesh (U.S. Standard) and loaded into 20 cm (8-inch) diameter, low carbon steel containers which were hot outgassed at 204°C (400°F) and then sealed by welding. The containers were then heated to 1185°C (2165°F) and isostatically compacted at this temperature for four hours at a pressure of 103.5 MPa (15 ksi) and then slowly cooled to ambient temperature. The resulting compacts were then heated to a temperature of 1121°C (2050°F), hot worked to 8 cm (3-inch) diameter bars, and finally annealed using a conventional high speed tool steel annealing cycle.

The commercial powder metallurgy tool steels were produced from -16 mesh nitrogen atomized powders and are representative of materials receiving different amounts of hot reduction after consolidation by hot isostatic pressing. No special measures were used in production of these steels to control sulfide size.

Several tests were conducted to compare the properties of the tool steel articles of the invention to those of articles made from high sulfur containing powder metallurgy tool steels of different manufacture. Tests were made to demonstrate the effects of composition and the methods of manufacture on sulfide size, bend fracture strength, impact strength, and machinability. The machinability tests were conducted on specimens in the fully annealed condition, whereas the bend fracture and impact tests were conducted on specimens in the hardened and tempered condition. The heat treatment for the latter specimens involved austenitizing for four minutes in molten salt at 1024°C (2200°F), oil quenching to room temperature, and triple tempering in molten salt for 2 hours plus 2 hours plus 2 hours at 552°C (1025°F). After this heat treatment, the hardness of the specimens ranged between 64 and 66 Rockwell C.

The sizes and distribution of the sulfides in the experimental and commercial tool steels are shown in Figures 1 and 2, respectively. As expected, the number of sulfides in experimental tool steels increase with sulfur content, as can be seen by comparing the microstructures for steels 92-17, 92-18, 92-19 and 92-20 in Figure 1. It is also clear that in accord with this invention all the sulfides in the experimental tool steels, regardless of sulfur content, are less than about 15 µm in their longest dimension. Further, it is clear that the size of the sulfides in the experimental tool steels are considerably smaller in their largest dimensions than the sulfides in the commercial tool steels of similar composition. As shown in Figure 2, the size of the sulfides in these latter steels range from about 20 to 30 µm in length, depending on the amount of hot reduction received in production.

The Charpy C-notch impact properties and bend fracture strengths of the experimental and commercial tool steels are given in Tables III and IV, respectively. Comparison of the results for the experimental tool steels shows that by keeping the maximum sulfide size below 15 µm, it is possible to increase sulfur content for the purpose of improving machinability without sacrificing toughness. This is indicated by the fact that the impact and bend fracture strengths of the experimental steels in both the longitudinal and transverse directions are essentially equivalent for sulfur contents ranging between 0.005 and 0.26%.

**Table III**

| IMPACT AND BEND FRACTURE STRENGTHS OF EXPERIMENTAL TOOL STEELS¹ | | | | | | | | |
|---|---|---|---|---|---|---|---|---|
| | | | | C-Notch Impact Strength (ft-lb) | | Bend Fracture Strength (ksi)x6.9=MPa) | | Maximum Sulfide Size microns |
| Bar Code | Sulfur Content | Hot Reduction | Hardness | Longitudinal | Transverse | Longitudinal | Transverse | |
| 92-17 | 0.004 | 85 | 66.5 | 24.0 | 9 | 757 | 517 | 4 |
| 92-18 | 0.05 | 85 | 66.0 | 25.5 | 11.5 | 753 | 507 | 6 |
| 92-19 | 0.14 | 85 | 66.0 | 23.0 | 11 | 139 | 547 | 12 |
| 92-20 | 0.26 | 85 | 65.0 | 24.0 | 11 | 711 | 561 | 15 |

**Table IV**

| IMPACT AND BEND FRACTURE STRENGTHS OF COMMERCIAL TOOL STEELS¹ | | | | | | | |
|---|---|---|---|---|---|---|---|
| | | | C-Notch Impact Strength (ft-lb) | | Bend Fracture Strength (ksi x 6.9=MPa) | | Maximum Sulfide Size microns |
| Bar Code | Hot Reduction % | Hardness HRC | Longitudinal | Transverse | Longitudinal | Transverse | |
| 92-79 | 60.5 | 65.0 | 9.0 | 4.5 | 411 | 369 | 28 |
| 92-81 | 60.5 | 64.5 | 10.0 | 6.0 | 559 | 389 | 20 |
| 92-77 | 85.0 | 65.0 | 18.5 | 5.5 | 672 | 421 | 24 |
| 92-78 | 85.0 | 65.0 | 19.0 | 5.5 | 651 | 383 | 32 |
| 92-72 | 94.0 | 66.0 | - | 7.0 | 655 | 391 | 30 |
| 92-74 | 94.0 | 66.0 | 19.5 | 8.0 | 695 | 427 | 30 |

| | | | | | | | |
|---|---|---|---|---|---|---|---|
| ¹ Austenitized at 1024°C (2200°F) for 4 minutes, oil quenched, and triple tempered at 552°C (1025°F) for 2 plus 2 plus 2 hours. | | | | | | | |

Comparison of the mechanical properties for the commercial tool steels given in Table IV shows that their impact and bend fracture strengths are generally improved by increasing the amounts of hot reduction, even though it results in some elongation of the sulfides. However, because of the larger size of the sulfides in these steels, their mechanical properties are significantly lower than those of the experimental tool steels having essentially the same composition and amount of hot reduction. Compare, for example, the mechanical properties of Steel 92-20 (0.26% S) which has a maximum sulfide size of about 15 µm and longitudinal and transverse bend fracture strengths of 5320 (771) and 3871 MPa (561 ksi), respectively, with those of Steel 92-78 (0.24% S) with a maximum sulfide size of about 30 µm and longitudinal and transverse bend fracture strengths of 4492 (651) and 2643 MPa (383 ksi), respectively.

The results of the drill machinability tests conducted on the experimental tool steels in the annealed condition are given in Table V. The drill machinability indexes in this table were obtained by comparing the times required to drill holes of the same size and depth in these steels and by multiplying the ratios of the times for each steel to that for the experimental steel with 0.005% sulfur by 100. Indexes greater than 100 indicate that the drill machinability of the steel being tested is greater than that of the experimental tool steel article containing 0.005% sulfur (Steel 91-60). The results show that increasing sulfur from 0.005 to 0.26% improves machinability of the experimental tool steels and that the greater improvement is achieved at sulfur contents at or above about 0.14%.

**Table V**

| EFFECT OF SULFUR CONTENT ON THE DRILL MACHINABILITY OF EXPERIMENTAL TOOL STEELS | | | | |
|---|---|---|---|---|
| Bar Number | % S | Hardness HRC | Drill Machinability Index-MI¹ | |
| | | | Test Values | Avg. |
| 91-17 | 0.005 | 21 | 100, 100, 100 | 100 |
| 91-18 | 0.05 | 21 | 104, 104, 109 | 106 |
| 91-19 | 0.14 | 22 | 117, 116, 127 | 120 |
| 91-20 | 0.26 | 21 | 140, 134, 150 | 141 |

| | | | | |
|---|---|---|---|---|
| ¹ Drill Machinability Index = $\frac{\text{Time to Drill Test Material}}{\text{Time to Drill Reference Standard Material}}$ x 100 | | | | |

It may be seen from the above that by reducing the size of the sulfides in articles made from hot worked powder metallurgy tool steels, it is possible to substantially negate the negative effects of high sulfur contents on their properties. Hence, with the invention it is possible to produce powder metallurgy tool steel articles with sulfur contents higher than conventionally permitted to achieve improved machinability without significant degradation of the mechanical properties, particularly as exhibited by the bend fracture strength of the steel.

The term "sulfur containing tool steel article" is restricted to cold work tool steels and high speed tool steels.

## Claims

1. A machinable powder metallurgy produced sulphur containing tool steel article comprising a hot worked, fully dense, consolidated mass of nitrogen gas atomized, prealloyed particles of a tool steel alloy, said tool steel alloy comprising in weight percent 0.80 to 3.00 carbon, 0.20 to 2.00 manganese, 0.10 to 0.30 sulphur, up to 0.04 phosphorus, 0.20 to 1.50 silicon, 3.0 to 12.00 chromium, 0.25 to 10.00 vanadium, up to 11.00 molybdenum, up to 18.00 tungsten, up to 10.00 cobalt, up to 0.10 nitrogen, up to 0.025 oxygen, balance iron and incidental impurities, characterised in that said article has a maximum sulphide size controlled to be less than about 15 µm.

2. A machinable powder metallurgy produced sulphur containing tool steel article having a minimum transverse bend fracture strength of 3450 MPa (500 ksi) when heat treated to hardness of 64 to 66 HRC, said article comprising a hot worked, fully dense, consolidated mass of nitrogen gas atomized, prealloyed particles of a tool steel alloy comprising, in weight percent, 1.25 to 1.50 carbon, 0.20 to 1.00 manganese, 0.10 to 0.26 sulphur, up to 0.04 phosphorus, up to 1.00 silicon, 3.0 to 6.00 chromium, 4.0 to 6.0 molybdenum, 3.50 to 4.50 vanadium, 4.0 to 6.5 tungsten, up to 0.025 oxygen, up to 0.10 nitrogen, balance iron and incidental impurities, characterised in that said article has a maximum sulphide size controlled to be less than about 15 µm.

3. A powder metallurgy produced sulphur bearing tool steel article of claim 1 or claim 2 in which the sulphur content is within the range of 0.14 to 0.26 percent.

4. A method for manufacturing a powder metallurgy sulphur containing tool steel article comprising a hot worked, fully dense, consolidated mass of nitrogen atomized, prealloyed particles of a tool steel alloy comprising, in weight percent 0.80 to 3.00 carbon, 0.20 to 2.00 manganese, 0.10 to 0.30 sulphur, up to 0.04 phosphorus, 0.20 to 1.50 silicon, 3 to 12.00 chromium, 0.25 to 10.00 vanadium, up to 11.00 molybdenum, up to 18.00 tungsten, up to 10.00 cobalt, up to 0.10 nitrogen, up to 0.025 oxygen, balance iron and incidental impurities, said article having a maximum sulphide size controlled to be less than about 15 µm, said method comprising producing said prealloyed particles by nitrogen gas atomization, hot isostatically compacting the prealloyed particles to full density at a temperature of 1185°C (2165°F) and a pressure of 103.5 MPa (15 ksi), hot working the resulting compact to a desired shape of the article at a temperature of 1121°C (2050°F), and annealing said article.

5. A method for manufacturing a powder metallurgy sulphur containing tool steel article having a minimum transverse bend fracture strength of 3450 MPa (500 ksi) when heat treated to hardness of 64 to 66 HRC, said article comprising a hot worked, fully dense, consolidated mass of nitrogen atomized, prealloyed particles of a tool steel alloy comprising, in weight percent, 1.25 to 1.50 carbon, 0.20 to 1.00 manganese, 0.10 to 0.26 sulphur, up to 0.04 phosphorus, up to 1.00 silicon, 3.0 to 6.0 chromium, 4.0 to 6.0 molybdenum, 3.5 to 4.50 vanadium, 4.0 to 6.5 tungsten, up to 0.025 oxygen, up to 0.10 nitrogen, balance iron and incidental impurities, said article having a maximum sulphide size controlled to be less than about 15 µm, said method producing said prealloyed particles by nitrogen gas atomization, compacting the prealloyed particles to full density at 1185°C (2165°F) and at a pressure of 103.5 MPa (15 ksi), hot working the compact to a desired shape of the article at a temperature of 1121°C (2050°F), and annealing said article.

6. The method of claims 4 or 5 in which the sulphur content is within the range of 0.14 to 0.26 weight percent.

## Patentansprüche

1. Bearbeitbarer, pulvermetallurgisch hergestellter, Schwefel enthaltender Werkzeugstahlgegenstand, der eine heiß bearbeitete, völlig dichte, konsolidierte Masse aus mit gasförmigem Stickstoff zerstäubten, vorlegierten Teilchen einer Werkzeugstahllegierung umfaßt, wobei diese Werkzeugstahllegierung in Gewichtsprozent 0,80 bis 3,00 Kohlenstoff, 0,20 bis 2,00 Mangan, 0,10 bis 0,30 Schwefel, bis zu 0,04 Phosphor, 0,20 bis 1,50 Silizium, 3,0 bis 12,00 Chrom, 0,25 bis 10,00 Vanadium, bis zu 11,00 Molybdän, bis zu 18,00 Wolfram, bis zu 10,00 Kobalt, bis zu 0,10 Stickstoff, bis zu 0,025 Sauerstoff enthält, wobei der Rest von Eisen und zufälligen Verunreinigungen gebildet wird, dadurch gekennzeichnet, daß der Gegenstand eine maximale Sulfidgröße aufweist, die so gesteuert ist, daß sie weniger als 15 µm beträgt.

2. Bearbeitbarer pulvermetallurgisch hergestellter, Schwefel enthaltender Werkzeugstahlgegenstand, der eine minimale Querbigungs-Bruchfestigkeit von 3450 MPa (500 ksi) besitzt, wenn er zur Erzielung einer Härte von 64 bis 66 HRC hitzebehandelt worden ist, wobei dieser Gegenstand eine heißbearbeitete, völlig dichte, konsolidierte Masse aus mit gasförmigem Stickstoff zerstäubten, vorlegierten Teilchen einer Werkzeugstahllegierung umfaßt, die in Gewichtsprozent 1,25 bis 1,50 Kohlenstoff, 0,20 bis 1,00 Mangan, 1,10 bis 0,26 Schwefel, bis zu 0,04 Phosphor, bis zu 1,00 Silizium, 3,0 bis 6,00 Chrom, 4,0 bis 6,0 Molybdän, 3,50 bis 4,50 Vanadium, 4,0 bis 6,5 Wolfram, bis zu 0,025 Sauerstoff, bis zu 0,10 Stickstoff umfaßt, wobei der Rest aus Eisen und zufälligen Verunreinigungen besteht, dadurch gekennzeichnet, daß der Gegenstand eine maximale Sulfidgröße besitzt, die so gesteuert ist, daß sie weniger als ungefähr 0,15 µm beträgt.

3. Pulvermetallurgisch hergestellter, Schwefel enthaltender Lagerstahl Gegenstand nach Anspruch 1 oder 2, bei dem der Schwefelgehalt im Bereich von 0,14 Prozent bis 0,26 Prozent liegt.

4. Verfahren zur Herstellung eines pulvermetallurgischen, Schwefel enthaltenden Werkzeugstahlgegenstandes, der eine heißbearbeitete, völlig dichte, konsolidierte Masse aus mit Stickstoff zerstäubten, vorlegierten Teilchen einer Werkzeugstahllegierung umfaßt, die in Gewichtsprozent 0,80 bis 3,00 Kohlenstoff, 0,20 bis 2,00 Mangan, 0,10 bis 0,30 Schwefel, bis zu 0,04 Phosphor, 0,20 bis 1,50 Silizium, 3 bis 12,00 Chrom, 0,25 bis 10,00 Vanadium, bis zu 11,00 Molybdän, bis zu 18,00 Wolfram, bis zu 10,00 Kobalt, bis zu 0,10 Stickstoff, bis zu 0,025 Sauerstoff umfaßt, wobei der Rest aus Eisen und zufälligen Verunreinigungen besteht, und wobei der Gegenstand eine maximale Sulfidgröße besitzt, die so gesteuert ist, daß sie weniger als ungefähr 15 µm beträgt, und wobei das Verfahren die Schritte umfaßt, daß die vorlegierten Teilchen durch Zerstäubung mit gasförmigem Stickstoff hergestellt werden, die vorlegierten Teilchen isostatisch bei einer Temperatur von 1185°C (2165°F) und einem Druck von 103,5 Mpa (15 ksi) heiß auf volle Dichte verdichtet werden, daß der sich ergebende verdichtete Körper bei einer Temperatur von 1121°C (2050°F) auf die gewünschte Form des Gegenstandes heiiß bearbeitet und der Gegenstand geglüht wird.

5. Verfahren zur Herstellung eines pulvermetallurgischen, Schwefel enthaltenden Werkzeugstahlgegenstandes, der eine minimale Querbiegungs-Bruchfestigkeit von 3450 MPa (500 ksi) besitzt, wenn er zur Erzielung einer Härte von 64 bis 66 HRC hitzebehandelt worden ist, wobei dieser Gegenstand eine heißbearbeitete, völlig dichte, konsolidierte Masse von mit Stickstoff zerstäubten, vorlegierten Teilchen einer Werkzeugstahllegierung enthält, die in Gewichtsprozent 1,25 bis 1,50 Kohlenstoff, 0,20 bis 1,00 Mangan, 0,10 bis 0,26 Schwefel, bis zu 0,04 Phosphor, bis zu 1,00 Silizium, 3,0 bis 6,0 Chrom, 4,0 bis 6,0 Molybdän, 3,5 bis 4,50 Vanadium, 4,0 bis 6,5 Wolfram, bis zu 0,025 Sauerstoff, bis zu 0,10 Stickstoff enthält, wobei der Rest aus Eisen und zufälligen Verunreinigungen besteht, und wobei dieser Gegenstand eine maximale Sulfidgröße besitzt, die so gesteuert ist, daß sie kleiner als ungefähr 15 µm ist, und wobei das Verfahren die Schritte umfaßt, daß vorlegierte Teilchen durch Stickstoff-Gaszerstäubung hergestellt und die vorlegierten Teilchen bei einer Temperatur von 1185 °C (2165°F) und einem Druck von 103,5 MPa (15 ksi) auf volle Dichte verdichtet werden, daß der verdichtete Körper bei einer Temperatur von 1121°C (2050°F) heiß bearbeitet wird, um die gewünschte Form des Gegenstandes zur erzielen, und das der Gegenstand geglüht wird.

6. Verfahren nach Anspruch 4 oder 5, bei dem der Schwefelgehalt in einem Bereich von 0,14 bis 0,26 Gewichtsprozent liegt.

## Revendications

1. Objet en acier à outil contenant du soufre produit par la métallurgie des poudres et usinable, comprenant une masse compactée totalement dense travaillée à chaud de particules préalliées atomisées par de l'azote gazeux d'un alliage d'acier à outils, ledit alliage d'acier à outils comprenant, en pourcentage en poids, 0,80 à 3,00 de carbone, 0,20 à 2,00 de manganèse, 0,10 à 0,30 de soufre, jusqu'à 0,04 de phosphore, 0,20 à 1,50 de silicium, 3,00 à 12,00 de chrome, 0,25 à 10,00 de vanadium, jusqu'à 11,00 de molybdène, jusqu'à 18,00 de tungstène, jusqu'à 10,00 de cobalt, jusqu'à 0,10 d'azote, jusqu'à 0,025 d'oxygène et le reste en fer et en impuretés inhérentes, caractérisé en ce que ledit objet a une dimension maximale de sulfures contrôlée pour être inférieure à environ 15 µm.

2. Objet en acier à outils contenant du soufre produit par la métallurgie des poudres et usinable ayant une résistance à la rupture en flexion transversale minimale de 3450 MPa (500 kpsi) lorsqu'il est traité à chaud à une dureté de 64 à 66 HRC, ledit objet comprenant une masse compactée totalement dense et travaillée à chaud de particules préalliées, atomisées par de l'azote gazeux d'un alliage d'acier à outils comprenant, en pourcentage en poids, 1,25 à 1,50 de carbone, 0,20 à 1,00 de manganèse, 0,10 à 0,26 de soufre, jusqu'à 0,04 de phosphore, jusqu'à 1,0 de silicium, 3,0 à 6,0 de chrome, 4,0 à 6,0 de molybdène, 3,50 à 4,50 de vanadium, 4,0 à 6,5 de tungstène, jusqu'à 0,025 d'oxygène, jusqu'à 0,10 d'azote et le reste en fer et en impuretés inhérentes, caractérisé en ce que ledit objet à une dimension maximale de sulfures contrôlée pour être inférieure à environ 15 µm.

3. Objet en acier à outils contenant du soufre produit par la métallurgie des poudres selon la revendication 1 ou la revendication 2, dans lequel la teneur en soufre est à l'intérieur de la fourchette de 0,14 à 0,26 %.

4. Procédé pour fabriquer un objet en acier à outils contenant du soufre produit par la métallurgie des poudres, comprenant une masse compactée totalement dense et travaillée à chaud de particules préalliées atomisées par de l'azote gazeux d'un alliage d'acier à outils, comprenant, en pourcentage en poids, 0,80 à 3,00 de carbone, 0,20 à 2,00 de manganèse, 0,10 à 0,30 de soufre, jusqu'à 0,04 de phosphore, 0,20 à 1,50 de silicium, 3,00 à 12,00 de chrome, 0,25 à 10,00 de vanadium, jusqu'à 11,00 de molybdène, jusqu'à 18,00 de tungstène, jusqu'à 10,00 de cobalt, jusqu'à 0,10 d'azote, jusqu'à 0,025 d'oxygène, le reste en fer et en impuretés inhérentes, ledit article ayant une dimension maximale de sulfures contrôlée pour être inférieure à environ 15 µm, ledit procédé comprenant les étapes suivantes : produire lesdites particules préalliées par atomisation par l'azote gazeux, compacter isostatiquement à chaud les particules préalliées à leur densité totale à une température de 1185°C (2165°F) et une pression de 103,5 MPa (15 kpsi), travailler à chaud la masse compacte résultante à la forme désirée de l'objet à une température de 1121°C (2050°F), et recuire ledit objet.

5. Procédé pour fabriquer un objet en acier à outils contenant du soufre produit par la métallurgie des poudres, ayant une résistance à la rupture en flexion transversale minimale de 3450 MPa (500 kpsi) lorsqu'il est traité à chaud à une dureté de 64 à 66 HRC, ledit objet comprenant une masse compactée totalement dense et travaillée à chaud de particules préalliées, atomisées par de l'azote, d'un alliage d'acier à outils comprenant, en pourcentage en poids, 1,25 à 1,50 de carbone, 0,20 à 1,00 de manganèse, 0,10 à 0,26 de soufre, jusqu'à 0,04 de phosphore, jusqu'à 1,0 de silicium, 3,0 à 6,0 de chrome, 4,0 à 6,0 de molybdène, 3,50 à 4,50 de vanadium, 4,0 à 6,5 de tungstène, jusqu'à 0,025 d'oxygène, jusqu'à 0,10 d'azote, le reste en fer et en impuretés inhérentes, ledit article ayant une dimension maximale de sulfure contrôlée pour être inférieure à environ 15 pm, ledit procédé comprenant les étapes suivantes : produire lesdites particules préalliées par atomisation par de l'azote gazeux, compacter les particules préalliées à une densité totale à 1185°C (2165°F) et à une pression de 103,5 MPa (15 kpsi), travailler à chaud la masse compactée à la forme désirée de l'objet à une température de 1121°C ((2050°F) et recuire ledit objet.

6. Procédé selon les revendications 4 ou 5, dans lequel la teneur en soufre est à l'intérieur de la fourchette de 0,14 à 0,26 % en poids.
